

S LAKE.

CASTING.

APPLICATION FILED DEC. 29, 1919.

1,374,855.

Patented Apr. 12, 1921.

Fig. 1.



Fig. 2.



Fig. 3.



INVENTOR.

Simon Lake  
by W. A. Finney

ATTORNEY.

# UNITED STATES PATENT OFFICE.

SIMON LAKE, OF MILFORD, CONNECTICUT.

## CASTING.

1,374,855.

Specification of Letters Patent. Patented Apr. 12, 1921.

Application filed December 29, 1919. Serial No. 348,074.

To all whom it may concern:

Be it known that I, SIMON LAKE, a citizen of the United States, residing at Milford, in the county of New Haven and State of Connecticut, have invented a certain new and useful Improvement in Castings, of which the following is a full, clear, and exact description.

This invention relates to the art of casting, and, more particularly, to a method of and apparatus for producing castings of a very fine, intricate and fragile nature.

The object of the invention is to provide a method and apparatus whereby faithful reproductions in metal or other plastic of such articles as flowers, twigs, insects and the like small and delicate articles may be made.

To this end the invention consists in surrounding the object to be reproduced with a mold forming material of suitable character, destroying the object within the mold, removing the thus destroyed object from the mold thus leaving a cavity forming a faithful impression of it therein, forcing fluid or plastic metal or other suitable material into the thus produced mold cavity so as to completely fill the same, and finally, after the plastic has set or solidified, removing the surrounding mold material; and the invention consists further in apparatus for performing this method, all as I will proceed now to explain and finally claim.

In the accompanying drawings illustrating the invention, in the several figures of which like parts are similarly designated, Figure 1 is a section taken in the plane of line 1—1, Fig. 2. Fig. 2 is a plan view of the apparatus for carrying out my method completely set up. Fig. 3 is a sectional view showing the manner of carrying out one step of my method.

It will be understood that the drawings are illustrative merely of one kind of apparatus for carrying out my method, it being possible that others might be designed to produce the desired result; but in the interest of clearness of the understanding of my invention reference will be had to the particular form of apparatus shown.

Referring to Fig. 3, a metallic cylinder 1, provided with a lining of suitable refractory material 2 which is a non-conductor of electricity, and screwthreaded at both ends 55 as at 3, is supported by means of a collar

4 threaded to one end, upon a suitable support or platform 5. In this cylinder is positioned the article 6 which it is desired to reproduce, here shown as a flower, by means of a particle of wax or the like easily melted substance 7 into which the stem is inserted, the leaves and petals being supported by means of threads 8 attached thereto and to a temporary supporting cross-bar 9. I consider it advisable, when the article to be reproduced is of a very fragile nature or its parts are very thin or tissue-like, to dip it into melted paraffin-wax or the like, before positioning it in the cylinder. This dipping will form a thin coating covering the entire 70 article, thereby giving it more body. Or the article may be frozen to give it rigidity.

After the article is properly positioned and supported, the cylinder is filled with a refractory, electrical-conducting material 75 10, see Fig. 1, in a fluid state, and for this purpose I have found that a mixture of plaster of Paris and graphite is quite suitable. I also consider "aquadag," a mixture of deflocculated Acheson graphite in water 80 in which it remains suspended, manufactured by the International Acheson Graphite Company, of Niagara Falls, New York, a suitable graphite for mixture with the plaster of Paris. This refractory material is 85 allowed to solidify to form a mold around the article 6. When the material has set sufficiently to allow the cylinder with the thus-formed mold to be moved, the cylinder is mounted, as shown in Figs. 1 and 2, in 90 heads 11 and 12 screwthreaded to receive the threaded ends of the cylinder, and provided with refractory linings 13, and stuffing-boxes 14 and 15 respectively, also lined with refractory material. 95

Through the stuffing-box 14 is inserted a tube 16, preferably of metal, connected by a tube 17 with a pump (not shown) which may be used to produce either pressure or a vacuum within the mold cavity, as will later appear. To this tube 16 is also connected one terminal 18 of an electric circuit, the other terminal 19 of which is connected with a hollow electrode 20, preferably of carbon, inserted through the other stuffing-box 15. 105 This electrode is adjustable by means of a yoke 21 through which it passes and to which it is secured by means of a set-screw 22, the yoke being supported upon the sleeved ends of thumb nuts 23 capable of 110

screw-adjustment upon rods 24 fixed to the head 12.

By the means just described the electrode 20 will be adjusted so that its inner end is 5 in contact with the refractory conducting material of the mold, and electric current switched on. Owing to the electrical resistance set up in the mold material, the mold will become heated to such a temperature as 10 to fuse any coating which may have been applied to the article therein, and to char the article itself and the threads 8 which were used to support it. The electric current is then switched off, and the pump is 15 operated to force air through tubes 17 and 16 and the openings left by the charred threads into the mold, whereby all the charred material is loosened from the mold and forced out of it through the opening in 20 the electrode 20, thereby leaving a mold cavity which is a true duplicate of the article which formerly filled it.

The depression formed by the removal of the particle of wax 7, combined with 25 the space caused by the thickness of the refractory lining 13 of head 15, forms a cavity 25 which is now filled with molten metal or other plastic in fluid form. When metal is used this is accomplished by introducing a rod 26 of the metal to be used 30 through the hollow electrode 20, switching on the current, and moving the electrode away from the mold to form an arc, the intense heat of which will melt the metal of 35 the rod. When sufficient molten metal has accumulated in the cavity 25, the electrode 20 is moved forward thereby displacing all air and gases from the mold cavity. In this operation it may be assisted by suction from 40 the pump connected with tubes 16 and 17. The rod 26 is now operated as a plunger by means of thumb-nuts 27 carried by a yoke 28 to which the end of rod 26 is fixed as by set-screw 29, the nuts 27 being threaded on 45 the rods 24 in a manner similar to the nuts 23. By moving rod 26 forward it will exert pressure upon the molten metal in cavity 25 and force it into all the interstices of the mold cavity, any surplus being forced out 50 of the openings formed by the threads 8; and this pressure may be augmented by operating the pump connected to tube 17 to create a vacuum in the mold.

It will be understood that the molten 55 metal will not be chilled and hence become sluggish upon entering the mold because the material thereof is at a high temperature due to the heating effect of the electric current passing through the material of the 60 mold.

In order to have a tight sliding fit between the rod 26 and the interior of the electrode 20, I provide a packing of plastic material of a suitable nature adapted to be 65 forced into an annular cavity 30 by the set-

screw 22, thus preventing the molten metal from backing out of the electrode past the rod 26 when pressure is applied.

If plastic other than molten metal be used, it may be introduced into the electrode 70 20 and then forced therefrom into the mold cavity by any suitable plunger.

Of course, the more minute the interstices of the mold cavity, the greater the pressure 75 on the plastic must be in order to have it fill them.

When the molding action is complete, the electric current is switched off and the mold with its casting allowed to cool, after which 80 the mold material may be removed.

It will be understood that various changes in the steps of my method, and in the method itself, and in the apparatus, may be made without departing from the spirit of the invention of the scope of the claims following. 85

What I claim is:—

1. A method of casting, comprising forming 90 a mold of electrical-conducting material around the article to be reproduced, destroying the article within the mold by the heat of an electric current passing through the mold material, removing the remains of the article, filling the mold cavity thus formed with a plastic substance, and removing the mold material. 95

2. A method of forming reproductions of articles destructible by heat, comprising forming an electrical-conducting mold around the article, destroying the article in the mold by the heat of an electric current 100 passing through the mold material, removing the remains of the thus destroyed article by introducing a fluid under pressure to the thus formed mold cavity, filling the mold cavity with plastic substance, and removing the mold. 105

3. A method of casting metal reproductions of articles, comprising forming a mold of electrical-conducting material around the article to be reproduced, passing an electric 110 current through said mold to heat the same and thereby char said article, removing the charred remains of the article by introducing a fluid under pressure to said mold to form a mold cavity, removing any gases remaining in said cavity, forcing molten metal into said cavity under pressure to fill the same, allowing the metal to cool, and removing the mold material from the casting thus formed. 115

4. In an apparatus for producing castings, a mold having electrical conducting properties and means for heating the same by passing an electric current through it, means for creating pressure or a vacuum therein, and means for introducing casting 120 material to said mold under pressure.

5. In an apparatus for producing metal and the like castings, means for forming a mold around the article to be reproduced, means for heating the mold by passing an 130

electric current therethrough to destroy the article, means for removing the remains of the article to form a cavity, and means for filling said cavity with plastic material.

5. 6. In an apparatus for producing castings, a mold of electrical conducting material formed around the article to be reproduced and containing same, means including electrical connections adapted to supply current for heating the material of the mold to char said article, means for introducing fluid under pressure to said mold to remove the charred remains of the article, and means for introducing molten metal to the mold
- 10 15 cavity thus formed.

7. In an apparatus for producing metal reproductions of articles destructible by heat, a mold of conducting material formed around and containing the article to be re-

produced, means for supplying electrical current to said mold to heat the same and destroy the article therein, means including one electrode of said current-supplying means for introducing compressed air to said mold to remove said destroyed article and thereby produce a mold cavity, and means including the other electrode of said current supplying means for producing an arc to melt metal and force the thus melted metal into said cavity under pressure. 30

In testimony whereof I have hereunto set my hand this 27th day of December, A. D. 1919.

SIMON LAKE.

Witnesses:

LUCY B. McLAUGHLIN,  
R. M. KEYS.